

April 3, 1928.

1,665,072

W. J. SCHENK

MANUFACTURE OF IMITATION MARBLE PANELS

Filed March 9, 1927



INVENTOR,  
W. J. Schenk;  
BY G. E. Maynard,  
ATTORNEY.

## UNITED STATES PATENT OFFICE.

WILLIAM J. SCHENK, OF HOME GARDENS, CALIFORNIA.

## MANUFACTURE OF IMITATION-MARBLE PANELS.

Application filed March 9, 1927. Serial No. 174,067.

This invention relates to composition panels for furniture construction.

An object of the invention is to provide a marble-like top or panel element for various pieces of furniture, and other uses.

Another object is to provide a simple, practicable and substantial built-up and artificial stone inlaid member.

Other objects, advantages and features will be made manifest in the following specification of the herewith illustrated embodiment and method; it being understood that modifications, variations and adaptations may be conceived and utilized within the spirit, scope and principle of the invention as it is more directly hereinafter claimed.

Figure 1 is a transverse section of a table top of the present invention; showing, also, a compressing tool.

Figure 2 is an edge view of the layer building process and layer sprinkling.

Figure 3 illustrates a roll of composition and its slicing.

In practicing my invention a composite member is made as follows:

A box or frame is made of bordering mold 2 having inner, echelon steps or shoulders 3 and 4 and upon the lower step 4 there is firmly glued, or otherwise secured, a stout 30 laminated bed (of wood veneer) 5. The top lip 6 of the frame thus made is dressed true to a common plane.

The recess above the bed 5 is filled with a plastic body of self-setting batch consisting of

|                           | Pounds. |
|---------------------------|---------|
| Magnesite                 | 30      |
| Celite                    | 4       |
| A. bleach                 | 6       |
| 40 Silica (150 mesh fine) | 40      |
| Talcum powder             | 4       |
| China clay                | 16      |

These ingredients are thoroughly mixed with a solution of magnesium chloride of 22 degrees specific gravity, to the consistency of bread dough.

A portion of this batch is spread out on a cloth covered plane to form a layer of say two feet in diameter and one-half inch in thickness (for a given size bed 5). Then a mineral color powder coat is thinly sprinkled over the laid batch and this is repeated by building up a suitable number of superposed layers, A, B, C, in Fig. 2, each having a color coat as at D, E, F, which vary in color or in tint as may be desired.

This body is then rolled up like a jelly roll, Fig. 3, and is sliced in transverse, longitudinal or oblique planes, in slices somewhat thicker than the depth of the recess over the bed 5.

The slices are laid flat and close as possible on the bed 5 and a heavy roller is rolled to and fro over the inlay M until this is well compacted.

The compressed inlay is then left to set for an hour or so, and the top is scraped to a smooth plane to bring out the beautiful hair lines of coloring matter which appear scattered throughout the inlay M from top to bottom in wholly indefinite lines.

The laminated bed 5 has the advantage over an integral bed piece (of wood) in that it will not warp and produce fracturing strains in the marble-like inlay.

The finally set inlay forms a very dense body with a nearly polished, finish exposed top face.

## What is claimed is:

The herein described method of manufacturing a marble-like panel which consists of making a magnesite cement, building a flat body of this in layers and applying a thin sprinkling of mineral coloring powder as each layer is formed, rolling the plastic body to give a spiral form to the layers, dividing the roll cross-wise into slices, laying the slices flat upon a framed panel back, compacting the slices to approximately the plane of the frame, and finally smoothing off the top of the filling flush with the frame edge and letting harden in the frame.

WM. J. SCHENK.